

## UNITED STATES PATENT OFFICE

2,613,131

PROCESS OF REDUCING THE CORROSION  
OF FERROUS METALS BY AMMONIACAL  
SOLUTION AND CORROSION INHIBITOR  
THEREFORMarion D. Barnes, Boyd L. Embrey, and Russell E.  
Koons, El Dorado, Ark., assignors to Lion Oil  
Company, El Dorado, Ark., a corporation of  
DelawareNo Drawing. Application October 27, 1950,  
Serial No. 192,628

18 Claims. (Cl. 23—1)

1

The present invention relates to a process of reducing corrosion, and more particularly to a process of reducing the corrosion of ferrous metals by ammoniacal solutions of nitrogen compounds, known in the trade as nitrogen solutions.

One large use of nitrogen solutions is in the manufacture of fertilizers. The present invention has particular application in the fertilizer industry. Nitrogen compounds involved in the manufacture of fertilizers include ammonium nitrate, sodium nitrate and urea. Of these, ammonium nitrate is perhaps the most important. The corrosiveness of nitrogen solutions is a very serious problem encountered in their manufacture, distribution and use. The solutions very rapidly corrode ferrous metal, e. g., mild steel, resulting in a severe metal loss, an accumulation of a greenish-black ferrous sludge which gradually turns into a reddish-brown precipitate of ferric oxide, and a severe cracking of the metal. Thus, equipment used in the manufacture, shipping and storage of nitrogen solutions is normally damaged beyond use within a few months or less.

Faced with this serious situation, industry has spent considerable time and money in research to minimize the problem. The corrosiveness of nitrogen solutions has been lessened by the addition thereto of various substances referred to in the art as corrosion inhibitors. Both single inhibitors and combinations of inhibitors have been employed. One possible function of these inhibitors is to deposit a protective coating on the metal with which the nitrogen solutions come in contact and thereby inhibit or decrease the corrosion of the metal by the solutions. Although progress has been made in this regard, the problem has not been solved satisfactorily. One chief disadvantage is that the corrosion rate, although materially inhibited, is still undesirably high. A further disadvantage is that the inhibitors heretofore used do not prevent the nitrogen solutions from becoming undesirably contaminated, e. g., by suspended corrosion products.

An object of this invention is to provide a process of reducing corrosion of ferrous metal by nitrogen solutions. A further object is to provide a process of reducing the corrosion of ferrous metal by nitrogen solutions, whereby the corrosion is reduced to a point substantially below that provided for heretofore. A still further object is to provide such a process which is further characterized by maintaining the nitrogen solutions remarkably clear. An additional object is to minimize the disadvantages of the prior

2

art. Other objects will be apparent from the description of this invention given hereinafter.

The above objects are accomplished according to this invention broadly by providing and practicing the process which comprises incorporating in a nitrogen solution a compound having an SH group and an OH group, the amount of the compound being sufficient to substantially reduce the rate of corrosion of a ferrous metal by the nitrogen solution, and contacting the solution with a ferrous metal.

While improved results are realized by incorporating alone in the nitrogen solution a compound having an SH group and an OH group, additional improved results to a remarkable extent are obtained by incorporating in addition to said compound an inorganic trivalent arsenic compound.

The degree to which the compounds having an SH group and an OH group keep the nitrogen solution clear is surprisingly high. The remarkable increase in effectiveness of these compounds in reducing the corrosion when used together with an inorganic trivalent arsenic compound is still more surprising. The compounds having an SH group and an OH group used alone proved to be relatively poor inhibitors but excellent in maintaining the nitrogen solution clear. These compounds in combination with an inorganic trivalent arsenic compound improved only very slightly in their ability to impart clearness to the nitrogen solution, but the combination proved to be a far better inhibitor than inhibitors heretofore used and also far better than would be expected, judging from their effect when used alone. Thus it appears that either a synergistic effect of a high order takes place or new compound formation takes place.

The number of compounds having an SH group and an OH group is comparatively small. Examples of such compounds include the following: 2-mercaptopropanol ( $\text{CH}_2\text{SHCH}_2\text{OH}$ ), 2,3-dimercaptopropanol-1 ( $\text{CH}_2\text{SHCH}_2\text{SHCH}_2\text{OH}$ ), 1-mercaptopropanol-2 ( $\text{CH}_3\text{CHOHCH}_2\text{SH}$ ), 1-mercaptopropanol-2 ( $\text{CH}_3\text{CH}_2\text{CHOHCH}_2\text{SH}$ ), 3-mercaptopropanol-1 ( $\text{CH}_2\text{SHCH}_2\text{CH}_2\text{OH}$ ), 2-mercaptopropanol-1 ( $\text{C}_6\text{H}_5\text{CHOHCH}_2\text{SH}$ ), 1-mercaptopropanol-2 ( $\text{CH}_2\text{SHCHOHCH}_2\text{CH}_3$ ),

1-mercaptopropane-2,3-diol

( $\text{CH}_2\text{OHCHOHCH}_2\text{SH}$ )

and isomers of said compounds. Of these compounds, 2-mercaptopropanol and 2,3-dimercaptopropanol are the most effective.

propanol-1 were substantially better than the others when used alone and particularly when used in combination with inorganic trivalent arsenic compounds. 2-mercapto ethanol was somewhat the better of the two compounds. The compounds listed, other than the first two, normally are not readily available commercially and are expensive to prepare.

The compounds containing OH and SH groups may be prepared by any of the methods available in the chemical literature but more commonly by the treatment of epoxides with hydrogen sulfide which brings about rupture of the epoxide ring and the introduction of an OH group and SH group respectively on the carbon atoms formerly joined through the oxygen atom of the epoxide ring. Alternatively compounds containing OH and SH groups may be prepared from compounds containing chlorine atoms and OH groups (e. g. chlorohydrins) by treating them with sodium sulfide, sodium hydrosulfide or other substance capable of yielding SH groups.

Inorganic trivalent arsenic compounds useful according to this invention include, e. g., sodium arsenite, potassium arsenite, ammonium arsenite, arsenic trioxide, and sulfides of trivalent arsenic. Of these, sodium arsenite was most used because of its ready availability and low cost. To increase the solubility of the inorganic trivalent arsenic compound in the nitrogen solution, desirably such compound will be dissolved in an alkali such as dilute sodium hydroxide.

In view of the foregoing and for the sake of clarity, this invention will be described for the most part with reference to employing 2-mercapto ethanol and sodium arsenite in combination as a corrosion inhibitor for substantially reducing the rate of corrosion of a ferrous metal by an ammoniacal ammonium nitrate solution, this being a preferred embodiment of the invention.

Ammoniacal ammonium nitrate solutions may vary considerably in composition. Fairly representative of such solutions encountered in industry and which give rise to the corrosion problem discussed hereinbefore are those having approximately 50%-75% ammonium nitrate, 15%-30% free ammonia and the remainder mostly water.

The quantity of inhibitor used is not critical over a fairly broad range and may vary upwards from a very low percentage of the nitrogen solution. Below about 0.005% inhibitor by weight of the nitrogen solution is not as effective as desirable. The upper limit is governed by economy. While about 1% by weight of the nitrogen solution may be used, the increased cost normally is not justified by the small improvement realized. The preferred range of inhibitor was found to be, by weight of the nitrogen solution, about 0.05%-0.1%.

The following example, wherein "parts" and "per cent" are by weight illustrates a specific embodiment of the present invention.

#### Example

354 parts of an ammoniacal ammonium nitrate solution, consisting of 66.8% ammonium nitrate and 16.6% anhydrous ammonia and 16.6% water, was placed in a closed container. The inhibitor was added and a test specimen of mild steel suspended freely in the nitrogen solution. The test specimens were weighed daily throughout the test period of 30 days and the corrosion reported as mg./cm.<sup>2</sup>/day weight loss.

In this particular example involving the addi-

tion of two inhibitors they were added separately to the ammonium nitrate solution, however they may be mixed prior to addition to the ammonium nitrate solution. The per cent sodium arsenite is calculated as arsenic trioxide (As<sub>2</sub>O<sub>3</sub>). The results obtained are tabulated below:

| Inhibitor                                      | Percent Inhibitor (Based on the Nitrogen Solution) | Corrosion mg./cm. <sup>2</sup> /day (Avg. for 30 days) |
|------------------------------------------------|----------------------------------------------------|--------------------------------------------------------|
| 2-mercapto ethanol                             | 0.1                                                | 0.157                                                  |
| Sodium arsenite                                | 0.1                                                | 0.175                                                  |
| Ammonium thiocyanate                           | 0.1                                                | 0.14                                                   |
| Butyl mercaptan                                | 0.1                                                | 0.16                                                   |
| 2-mercapto ethanol and sodium arsenite         | 0.05 of each                                       | 0.01                                                   |
| Ammonium thiocyanate and sodium arsenite       | { 0.1<br>0.05 }                                    | 0.19                                                   |
| Butyl mercaptan and sodium arsenite            | 0.1 of each                                        | 0.13                                                   |
| 2, 3-dimercapto propanol-1 and sodium arsenite | { 0.1<br>0.05 }                                    | 0.06                                                   |

A control test (blank) was run according to the above procedure except that no inhibitor was used. After only 5 hours in the uninhibited ammoniacal ammonium nitrate solution, the weight loss of the test specimen was 34.4 mg./cm.<sup>2</sup>. On this basis the corrosion rate of the uninhibited solution on the test specimen was 162.7 mg./cm.<sup>2</sup>/day.

It will be understood that the foregoing example is merely illustrative and does not limit the present invention, which more broadly comprises incorporating in a nitrogen solution a compound having an SH group and an OH group, the amount of said compound being sufficient to substantially reduce the rate of corrosion of a ferrous metal by the solution, and contacting said solution with said ferrous metal.

In carrying out this invention according to a preferred embodiment thereof indicated hereinbefore, to a nitrogen solution in a railroad tank car (or storage, conveying, measuring, and other handling equipment) are added 0.1% of 2-mercapto ethanol and 0.05% sodium arsenite by weight of the nitrogen solution. This substantially reduces the rate of corrosion of the metal equipment by the nitrogen solution and maintains the solution very clear for approximately thirty days. For at least the next fifteen days these desirable results are still achieved but to a lesser extent. Although it is not definitely known how the nitrogen solution is kept clear in spite of the formation of corrosion products, such as oxides of iron, there is reasonably strong evidence that the inhibitor dissolves these products and when so dissolved they are substantially colorless.

From the example set forth hereinbefore, it will be seen that when 2-mercapto ethanol was used alone its effect in reducing the corrosion was practically the same as conventional inhibitors such as sodium arsenite, ammonium thiocyanate and butyl mercaptan. However, 2-mercapto ethanol used alone was far superior to conventional inhibitors in maintaining the nitrogen solution clear. When 2-mercapto ethanol was combined with sodium arsenite, this superiority in clarity of the nitrogen solution again resulted, and the corrosion-inhibiting power of the combination was many times better than either of these two compounds used separately or the sum of their separate effects—a vast synergistic effect. Similar combinations of conventional inhibitors did not exhibit synergism to any material degree.

The reason for this synergism is not known. While it is not intended to limit this invention to any theory by way of one possible explanation there is some evidence that compounds containing an OH group and an SH group (e. g. 2-mercapto ethanol) react with inorganic trivalent arsenic compounds (e. g. sodium arsenite) to produce a new compound, and actually the new compound produces the desired result. This evidence consists of the observation that a large amount of heat is liberated when 2-mercapto ethanol is added to sodium arsenite, and that, in addition to temperature increase, hydrogen sulfide gas is liberated when 2-mercapto ethanol is added to sodium thioarsenite.

As many apparently widely different embodiments of this invention may be made without departing from the spirit and scope thereof, it is to be understood that the invention is not limited to the specific embodiments thereof except as defined in the appended claims.

What is claimed is:

1. Process of reducing corrosion of a ferrous metal by an ammoniacal solution of a nitrogen compound, which comprises incorporating in said solution a compound having an SH group and an OH group together with an inorganic trivalent arsenic compound, the amounts of said compounds being sufficient to substantially reduce the rate of corrosion of a ferrous metal by the solution, and contacting said solution with said ferrous metal.

2. Process of reducing corrosion of a ferrous metal by an ammoniacal ammonium nitrate solution, which comprises incorporating in said solution a compound having an SH group and an OH group together with an inorganic trivalent arsenic compound, the amounts of said compounds being sufficient to substantially reduce the rate of corrosion of a ferrous metal by the solution, and contacting said solution with said ferrous metal.

3. Process of reducing corrosion of a ferrous metal by an ammoniacal solution of a nitrogen compound, which comprises incorporating in said solution an inorganic trivalent arsenic compound together with a compound selected from the group consisting of 2-mercapto ethanol and 2,3-dimercapto propanol-1, the amounts of said compounds being sufficient to substantially reduce the rate of corrosion of a ferrous metal by the solution, and contacting said solution with said ferrous metal.

4. Process of reducing corrosion of a ferrous metal by an ammoniacal solution of a nitrogen compound, which comprises incorporating in said solution sodium arsenite together with a compound selected from the group consisting of 2-mercapto ethanol and 2,3-dimercapto propanol-1, the amounts of said compounds being sufficient to substantially reduce the rate of corrosion of a ferrous metal by the solution, and contacting said solution with said ferrous metal.

5. Process of reducing corrosion of a ferrous metal by an ammoniacal solution of a nitrogen compound, which comprises incorporating in said solution 0.005%-1% of an inorganic trivalent arsenic compound together with 0.005%-1% of a compound selected from the group consisting of 2-mercapto ethanol and 2,3-dimercapto propanol-1, the amounts of said compounds being by weight of said solution and sufficient to substantially reduce the rate of corrosion of a ferrous metal by the solution, and contacting said solution with said ferrous metal.

6. Process of reducing corrosion of a ferrous metal by an ammoniacal ammonium nitrate solution, which comprises incorporating in said solution sodium arsenite and 2-mercapto ethanol, the amounts of said compounds being sufficient to substantially reduce the rate of corrosion of a ferrous metal by the solution, and contacting said solution with said ferrous metal.

7. Process of reducing corrosion of a ferrous metal by an ammoniacal ammonium nitrate solution, which comprises incorporating in said solution 0.05%-0.1% of sodium arsenite and 0.05%-0.1% of 2-mercapto ethanol, the amounts of said compounds being by weight of said solution and sufficient to substantially reduce the rate of corrosion of a ferrous metal by the solution, and contacting said solution with said ferrous metal.

8. Process of reducing corrosion of a ferrous metal by an ammoniacal ammonium nitrate solution, which comprises incorporating in said solution sodium arsenite and 2,3-dimercapto propanol-1, the amounts of said compounds being sufficient to substantially reduce the rate of corrosion of a ferrous metal by the solution, and contacting said solution with said ferrous metal.

9. Process of reducing corrosion of a ferrous metal by an ammoniacal ammonium nitrate solution, which comprises incorporating in said solution 0.05%-0.1% of sodium arsenite and 0.05%-0.1% of 2,3-dimercapto propanol-1, the amounts of said compounds being by weight of said solution and sufficient to substantially reduce the rate of corrosion of a ferrous metal by the solution, and contacting said solution with said ferrous metal.

10. A non-corrosive liquid comprising an ammoniacal solution of a nitrogen compound, a compound having an SH group and an OH group and an inorganic trivalent arsenic compound, the amounts of said compounds being sufficient to substantially reduce the rate of corrosion of a ferrous metal by said solution.

11. A non-corrosive liquid comprising an ammoniacal ammonium nitrate solution, a compound having an SH group and an OH group and an inorganic trivalent arsenic compound, the amounts of said compounds being sufficient to substantially reduce the rate of corrosion of a ferrous metal by said solution.

12. A non-corrosive liquid comprising an ammoniacal solution of a nitrogen compound, an inorganic trivalent arsenic compound, and a compound selected from the group consisting of 2-mercapto ethanol and 2,3-dimercapto propanol-1, the amounts of said compounds being sufficient to substantially reduce the rate of corrosion of a ferrous metal by said solution.

13. A non-corrosive liquid comprising an ammoniacal solution of a nitrogen compound, 0.005%-1% of an inorganic trivalent arsenic compound, and 0.005%-1% of a compound selected from the group consisting of 2-mercapto ethanol and 2,3-dimercapto propanol-1, the amounts of said compounds being by weight of said solution and sufficient to substantially reduce the rate of corrosion of a ferrous metal by said solution.

14. A non-corrosive liquid comprising an ammoniacal ammonium nitrate solution, sodium arsenite and 2-mercapto ethanol, the amounts of said compounds being sufficient to substantially reduce the rate of corrosion of a ferrous metal by said solution.

15. A non-corrosive liquid comprising an ammoniacal ammonium nitrate solution, 0.05%-

0.1% of sodium arsenite and 0.05%-0.1% of 2-mercapto ethanol, the amounts of said compounds being by weight of said solution and sufficient to substantially reduce the rate of corrosion of a ferrous metal by said solution.

16. A non-corrosive liquid comprising an ammoniacal ammonium nitrate solution, 0.05%-0.1% of sodium arsenite and 0.05%-0.1% of 2-mercapto ethanol, the amounts of said compounds being by weight of said solution and sufficient to substantially reduce the rate of corrosion of a ferrous metal by said solution, said solution including by weight thereof approximately 50%-75% ammonium nitrate, 15%-30% free ammonia and the remainder mostly water.

17. A non-corrosive liquid comprising an ammoniacal ammonium nitrate solution, sodium arsenite and 2,3-dimercapto propanol-1, the amounts of said compounds being sufficient to substantially reduce the rate of corrosion of a ferrous metal by said solution.

18. A non-corrosive liquid comprising am-

moniacal ammonium nitrate solution, 0.05%-0.1% of sodium arsenite and 0.05%-0.1% of 2,3-dimercapto propanol-1, the amounts of said compounds being by weight of said solution and sufficient to substantially reduce the rate of corrosion of a ferrous metal by said solution.

MARION D. BARNES.  
BOYD L. EMBREY.  
RUSSELL E. KOONS.

## REFERENCES CITED

The following references are of record in the file of this patent:

## UNITED STATES PATENTS

| Number    | Name                  | Date           |
|-----------|-----------------------|----------------|
| 2,198,151 | Beekhuis et al. ----- | Apr. 23, 1940  |
| 2,215,077 | Beekhuis et al. ----- | Sept. 17, 1940 |
| 2,215,092 | Beekhuis et al. ----- | Sept. 17, 1940 |
| 2,220,059 | Beekhuis et al. ----- | Nov. 5, 1940   |
| 2,238,651 | Keenen -----          | Apr. 15, 1941  |